

## UNITED STATES PATENT OFFICE

2,357,885

## MELTING MAGNESIUM

Russell Franks and William O. Binder, Niagara Falls, N. Y., assignors to Electro Metallurgical Company, a corporation of West Virginia

No Drawing. Application December 8, 1943,  
Serial No. 513,460

8 Claims.

(CL 75—67)

This invention relates to the melting of magnesium and magnesium-base alloys and refers more particularly to containers for holding such materials in the molten condition.

A disadvantage of magnesium and its alloys which has hindered their use as structural materials for some purposes is their susceptibility to localized corrosion, generally believed to be due to impurities. Impurities are ordinarily introduced during melting operations in the manufacture of magnesium alloys or in the fabrication of useful articles from magnesium and its alloys. The impurities thought to have the most damaging effect on the corrosion resistance of magnesium alloys are iron and nickel.

It is the commercial practice to employ carbon steel containers for handling and holding molten magnesium and magnesium-base alloys during their manufacture or fabrication. It has been observed that magnesium and magnesium-base alloys so handled may have quite poor resistance to corrosion despite the fact that magnesium of very high purity is used, but no commercially practicable alternative to this practice has heretofore been advanced.

It is the principal object of this invention to provide improved containers for holding and handling molten magnesium and its alloys, by the use of which containers metal having good resistance to corrosion may be produced. Other important objects of the invention include improvements in the method of melting magnesium and magnesium-base alloys and in methods of handling such materials in the molten condition.

The invention by which these objects are achieved is based on the discovery that molten magnesium and its alloys may be held in contact with certain steels, the principal characteristic of which is a high manganese content, without seriously detrimentally affecting their resistance to corrosion. The invention comprises a container for molten magnesium and magnesium alloys, which container is composed of a steel containing 10% to 30% manganese, the principal part of the remainder being iron. The steel of which the container of the invention is composed preferably also contains up to 18% chromium and may contain up to about 2% or somewhat more silicon, up to 1.5% carbon, up to 2% columbium, up to 1% copper, up to 2% molybdenum, up to 3% nickel, and up to about 0.3% nitrogen, and the incidental impurities commonly present in steels of good quality. The invention also comprises the improved methods of melting magnesium and its alloys and handling the molten

materials which include the step of conducting such operations in containers composed of such steels.

The composition of the steel used for containers for molten magnesium and its alloys in accordance with the invention may vary widely within the composition limits given. For example, containers may be composed of a steel containing 10% to 15% manganese and 0.8% to 1.5% carbon. If a steel containing more manganese, say about 16% to 30%, is used, the carbon content is preferably diminished and should not be more than about 0.5%. For containers more resistant to oxidation and loss of toughness at the elevated temperatures at which they are used, a steel containing up to 18% chromium, preferably 5% to 15% chromium, may be used. The presence of columbium up to about 2% or molybdenum up to about 2%, or both, improves the high temperature strength of the steel. Preferably, not more than 1% each of columbium or molybdenum is present, and steels containing these elements should contain less than 0.3% carbon. Small quantities of copper and of nickel may be present but the nickel content should not exceed about 3% nor the copper about 1%. Nitrogen in an amount not exceeding about 0.3% and preferably 0.05% to 0.15%, may be present in all of these steels as may be silicon, but the silicon content is preferably under 2%.

The corrosion-resistance of magnesium which has been melted in containers fabricated from the steels just described is markedly superior to the corrosion-resistance of magnesium, otherwise identical, which has been melted in containers composed of ordinary carbon steels. This conclusion is supported by the results of numerous tests in which several different samples of commercially pure magnesium were melted in different containers embodying the invention and in carbon steel containers under comparable melting conditions. Cast samples of the magnesium melted in these containers were subjected to corrosion tests in which the samples were exposed alternately to a 3% sodium chloride solution for a few minutes and to air for a few minutes, the alternate exposures being repeated and continued for a period of several days. In general, samples produced from the first one or two batches of magnesium melted in a given container had poor corrosion-resistance, but samples produced from successive batches melted in the same containers had markedly improved corrosion-resistance except in the case of samples produced from metal which had been melted in

carbon steel containers. Typical test results are shown in the following table in which the corrosion rate of samples taken from successive batches of pure magnesium melted in containers having the composition indicated is expressed as loss of weight in milligrams per square centimeter per day.

| Composition of container (remainder substantially all iron) | Batch number | Corrosion rate  |
|-------------------------------------------------------------|--------------|-----------------|
|                                                             |              | Mg./sq. cm./day |
| 0.2% C                                                      | 2            | 112             |
| Do                                                          | 3            | 63              |
| Do                                                          | 4            | 88              |
| 12% Mn; 1.2% C                                              | 2            | 7               |
| Do                                                          | 3            | 3               |
| Do                                                          | 4            | 0.5             |
| Do                                                          | 5            | 0.6             |
| Do                                                          | 6            | 0.6             |
| 18% Mn; 0.2% C                                              | 2            | 20              |
| Do                                                          | 3            | 1.5             |
| Do                                                          | 4            | 8               |
| Do                                                          | 5            | 2               |
| Do                                                          | 6            | 4               |
| 18% Mn; 2% Si; 0.2% C                                       | 2            | 37              |
| Do                                                          | 3            | 0.48            |
| Do                                                          | 4            | 0.32            |
| 20% Mn; 5% Cr; 2.0% Si; 0.15% C                             | 2            | 33              |
| Do                                                          | 3            | 0.84            |
| Do                                                          | 4            | 0.33            |
| 18% Mn; 13% Cr; 0.15% C                                     | 2            | 0.40            |
| Do                                                          | 3            | 0.35            |
| Do                                                          | 4            | 0.34            |
| Do                                                          | 5            | 0.36            |
| Do                                                          | 6            | 0.48            |
| 20% Mn; 12% Cr; 0.2% C                                      | 2            | 0.25            |
| Do                                                          | 3            | 0.33            |
| Do                                                          | 4            | 0.46            |
| Do                                                          | 5            | 0.33            |
| Do                                                          | 6            | 0.31            |
| 25% Mn; 13% Cr; 0.15% C                                     | 2            | 0.72            |
| Do                                                          | 3            | 0.25            |
| Do                                                          | 4            | 0.30            |

The improved corrosion-resistance of substantially pure magnesium melted in the containers of the invention, as compared with that of the same material melted in carbon steel containers is evident from the above table. Similar results were obtained in tests conducted using several of the well known magnesium alloys now in commercial use containing manganese and aluminum, some with and some without zinc, such alloys exhibiting substantially the same order of improvement in corrosion-resistance when melted in the containers of the invention as that shown by the substantially pure magnesium.

To attain the benefits of the invention, containers composed of the steel described should be employed whenever magnesium and its alloys are melted or are handled in the molten condition. By melting such materials and by handling them in the molten condition exclusively in such containers, the production of magnesium and magnesium-base alloys having greatly improved resistance to corrosion is achieved without changing substantially the composition of the materials now used commercially.

It is common practice in melting magnesium and its alloys to conduct the melting operation under a protective flux blanket. A relatively fluid flux is employed for some melting methods,

and a more viscous flux for others. The containers of the invention may be used for any type of melting procedure, with or without flux. In the melting operations reported in the above table, a viscous flux containing about 30% potassium chloride, 21% magnesium chloride, 19% calcium chloride, 12% magnesium fluoride, 7% calcium fluoride and 7% sodium chloride was used.

10 We claim:

1. In the art of handling molten magnesium and magnesium-base alloys, the improvement which comprises holding such molten materials in a container made of steel containing 10% to 30% manganese.

15 2. In the art of melting magnesium and magnesium-base alloys, the improvement which comprises melting such materials in a container composed of a steel containing 10% to 30% manganese.

20 3. In the art of melting magnesium and magnesium-base alloys, the improvement which comprises melting such materials in a container composed of a steel containing 10% to 30% manganese and up to about 18% chromium.

25 4. In the art of melting magnesium and magnesium-base alloys, the improvement which comprises melting such materials in a container composed of a steel containing 10% to 25 manganese, 12% to 15% chromium, up to about 2% each of columbium and silicon, up to about 1% of copper, up to about 2% of molybdenum, carbon in an amount not exceeding about 0.3%, the remainder substantially all iron.

30 5. A container for use in contact with molten magnesium and magnesium-base alloys which container is composed of a steel containing about 10% to 30% manganese.

35 6. A container for use in contact with molten magnesium and magnesium-base alloys which container is composed of a steel containing about 10% to 15% manganese, up to about 2% silicon, and 0.8% to 1.5% carbon.

40 7. A container for use in contact with molten magnesium and magnesium-base alloys which container is composed of a steel containing about 10% to 30% manganese, chromium in an amount up to about 18%, and the remainder principally iron.

45 8. A container for use in contact with molten magnesium and magnesium-base alloys which container is composed of a steel containing about 10% to 25% manganese, about 5% to 15% chromium, up to about 2% silicon, up to about 2% columbium, up to about 1% copper, up to about 2% molybdenum, nitrogen in an amount not exceeding about 0.15%, the remainder substantially all iron and incidental impurities including nickel, the nickel content not exceeding 3%.

RUSSELL FRANKS.  
WILLIAM O. BINDER.